

March 21, 1933.

D. W. HOGE

1,902,125

MOTOR FUEL

Original Filed Dec. 19, 1928 2 Sheets-Sheet 1



Fig. 1.

Inventor  
Daniel W. Hoge

*Daniel W. Hoge*  
Attorney

March 21, 1933.

D. W. HOGE

1,902,125

## MOTOR FUEL

Original Filed Dec. 19, 1928 2 Sheets-Sheet 2

Fig. 2.



*Inventor*

*Daniel W. Hoge*

*Daniel W. Roche*  
*James T. Ballew*  
*Attorney.*

Attorney.

## UNITED STATES PATENT OFFICE

DANIEL W. HOGE, OF LOS ANGELES, CALIFORNIA, ASSIGNOR TO CARLOS W. NEWBERRY,  
OF LOS ANGELES, CALIFORNIA

## MOTOR FUEL

Continuation of application Serial No. 327,013, filed December 19, 1928. This application filed July 20, 1929. Serial No. 379,810.

This invention has reference to fuels for internal combustion engines and more particularly to a motor fuel derived from constituents of crude turpentine, this material in addition to being highly superior as a fuel, having properties which render it capable of suppressing detonation when used alone as a motor fuel or when mixed with gasoline.

It is a purpose of the invention to produce by the destructive distillation or cracking of crude turpentine, which, disregarding impurities, is essentially a solution of rosin in oil of turpentine, or by the cracking of either of these constituents, preferably the rosin, a product or series of compounds of aromatic nature differing characteristically in specific gravity and boiling range, and of which a certain range is particularly suited for use as motor fuel. Typical processes by which the present product may be obtained are described in my copending application, of which the present application is a continuation, entitled Method for treating resins, Serial No. 327,013, filed December 19, 1928. In speaking of crude turpentine hereinafter it will be understood that I refer to the resinous exudate as obtained in the crude state from species of pine and comprising rosin and oil of turpentine, or to refined crude turpentine from which impurities such as foreign solids and water have been removed. Oil of turpentine, obtained commercially by the steam distillation of crude turpentine from which the comparatively non-volatile rosin remains as a residue, and also wood turpentine obtained by distillation from dead wood, and which may also be treated to obtain the present product, consist mainly of the hydrocyclic pinenes, and have close boiling ranges from about 310 to 350° F. The residual solid rosin or colophony remaining after distillation of oil of turpentine from the crude turpentine, consists mainly of abietic acid having a melting point around 300° F., and cannot be distilled at normal pressure without undergoing extensive decomposition, the distillate instead of solidifying, being in the form of an oily liquid known commercially as rosin oil. The latter has a comparatively broad boiling range, say from

100 to 700° F., and comprises a complex mixture of compounds, some of which are of the aromatic series, in addition to a considerable amount of organic acids. The bulk of the constituents of rosin oil however cannot be considered aromatic in nature due to insolubility of a considerable percentage of the oil in concentrated sulphuric acid, and in which aromatic compounds characteristically are soluble. Thus it may be noted at this point that by the mere heating and vaporizing of rosin, although in this operation cracking occurs to a certain degree, the cracking reaction does not take place to such an extent as to substantially convert the distillate into compounds of aromatic nature or compounds possessing the properties of aromatics.

In order to obtain products of the nature comprising the invention, turpentine or rosin is subjected to cracking to such an extent as to convert the distillate almost entirely into aromatic or kindred compounds, this being indicated by the fact that a typical distillate is found to dissolve at normal temperatures to the extent of 94% or more in concentrated sulphuric acid. Also the products are comparatively free of organic acids, this probably being due to the temperature of the cracking operation being sufficiently high to break down the carboxyl groups characteristic of the acidic compounds. As will be later noted, a comparison of the specific gravities and boiling points of the products gives further evidence of their being aromatic in nature.

The product embodied in the invention may be obtained as will later be described, from the above mentioned constituents of crude turpentine, preferably the rosin, and has such characteristics as to render it highly superior for use as motor fuel. Although the product finds its present and most general use as a non-detonating motor fuel and will be described as such, it will be understood that the invention in its broader aspects is not limited to the use of the product for this specific purpose, and in general it may be stated that the product is capable of numerous uses kindred to those of aromatic compounds such as benzol and toluol. Also, in

addition to the use of the present product by itself as motor fuel, the invention broadly contemplates the admixing of the present product with common motor fuels to render them non-detonating.

Typically and preferably, the present motor fuel is given a distillation range of or within say 100 to 450° F., roughly corresponding to the boiling range limits of the various grades of commercial gasoline. It will be understood of course that the boiling range of the fuel made under certain conditions vary somewhat beyond these limits, or it may be desired to give to the product a comparatively closer boiling range within these limits under other conditions, the temperatures given therefore representing the usual and typical maximum boiling range characteristic of the usual motor fuels. As a result of a series of tests made on the fuel, it is found to have a heating value around 21,400 B. T. U. per pounds, approximately 1000 B. T. U.'s higher than ordinary gasoline, these tests further indicating that substantially increased mileage may be had over that obtainable with gasoline, by the use of this fuel. This feature is of great importance with reference to the use of the fuel in airplanes, since it is essential that the maximum mileage be obtained from a given quantity of fuel, especially in cases where the duration of the flight may be determined by the amount of fuel that can be carried. Tests made on the product in motors specially equipped for determining the anti-knock character of fuel indicate that although motors may be operated under extremely severe conditions and under heavy loads, detonation is substantially entirely suppressed. Similar tests have shown the product to have non-detonating properties to a high degree that cannot be given to gasoline even by its treatment with known anti-knock compounds such as tetra-ethyl-lead. It is understood that increasing amounts of for instance tetra-ethyl-lead, when added to gasoline, serve to increase its non-detonating properties up to certain degree, but that beyond that point the tetra-ethyl-lead appears to have little effect in suppressing further detonation. Thus in the operation of some types of motors under extremely severe conditions, it has heretofore been impossible to prevent knocking by the use of gasoline rendered non-detonating to the highest possible degree by the use of certain common anti-knock reagents.

It is found that the present fuel is substantially the equivalent of benzol in its non-detonating properties, and as is well known, benzol is among the most effective of known materials for suppressing detonation. Approximately 16% of volume of the product mixed with gasoline is the equivalent of about 1.8 cc. of ethyl fluid per gallon of gasoline this being about the usual amount of the lead

compound used, although as previously mentioned, by increasing the proportion of the present material, the anti-knock properties of the fuel mixture will be increased accordingly, whereas a limit is reached at a comparatively lesser degree by increasing the amounts of the other. By the use of benzol as a non-detonating compound results similar to those obtained by the addition of the present product would be obtained, the high cost of benzol, however, preventing its use for this purpose whereas the present material may be produced at a comparatively low cost.

In carrying out the preferred method of obtaining the product, turpentine or rosin is subjected to vaporization and the vapors heated to a cracking temperature preferably between 600 and 1200° F., the cracked vapors then being fractionated by any well known means to give a product having the desired volatility range and physical characteristics. A typical apparatus for carrying out this method of production as well as the nature of the properties of the product comprising the invention, will be discussed to best advantage in the following detailed description, throughout which reference is had to the accompanying drawings, in which:

Figure 1 is a diagrammatic illustration of the preferred apparatus for carrying out the process by which the product is obtained; and

Fig. 2 is a graphic illustration of the boiling point curves plotted from tests of representative samples of distillates obtained from rosin and oil of turpentine.

Due to the availability of large quantities of rosin at comparatively low cost and which are obtained in the nature of a by-product in the extraction of oil of turpentine from the crude turpentine, the production of the fuel from rosin appears to have the greatest economic possibilities. And therefore during the following discussion, the product will be described mainly with reference to its production from rosin. It will be understood that I refer here to all rosins of this nature regardless of the method employed in their production and their sources, for example whether they be obtained from the exudate from living coniferae, or by distillation from dead trees and stumps.

Referring first to Fig. 1, the evaporator or still 10 is charged with rosin in solid form and fired to a temperature sufficient to vaporize the charge, the vapors (vaporized rosin oil) being conducted through line 11 to the tubular superheater which preferably is of the type described in my copending application No. 291,712 filed July 11, 1928. Upon flowing through the superheater, the vapors are heated to a temperature between 600 and 1200° F., and preferably around 900° F., at which temperature the vapors are thermally decomposed or cracked to form com-

pounds characterized in one respect by their higher boiling point, as will later be noted. The cracked vapors from the superheater are conducted through line 13 to the fractionating tower 14, a suitable trap 15 being placed in the vapor line to remove any liquid or carbonaceous bodies that may be carried in the vapor stream, and the materials in the trap being returned to the still 10 through line 16. The fractionating tower 14 is typical of any suitable means for obtaining from the cracked vapors a product having the desired predetermined boiling range. The cracked vapors from the superheater pass upwardly through the fractionating tower 14, a portion of the outlet vapor in line 17 being condensed in the condenser 18 and returned to the tower as reflux, and the liquid product being drawn off from the tower through line 19, at a predetermined point according to the volatility range which it is desired to give to the product. Thus in the present instance, the product fraction removed from the fractionating tower 14 through line 19 has a volatility range of substantially 100 to 450° F. The higher boiling point fractions are removed at the base of the tower through line 20, the final extremely volatile vapors or fixed gases being condensed in the condenser 21. In a typical run, the total yield of distillate from the rosin charge in the still 11 was approximately 70% by weight of the charge, although this figure may be materially increased since the still charge was not reduced to a minimum.

During a test run, the entire distillate, including the lightest and heaviest fractions, obtained from cracking about 850 lbs. of rosin was collected, and representative samples of the distillate taken at different times. Two of these samples were fractionally distilled in a common laboratory Hempel column, the temperature of the vapors being noted as each 5% fraction was collected, and the specific gravity of each fraction determined. These data appear in the two curves indicated in Figure 2, the boiling point of the end of the 5% fractions being plotted against their specific gravities. The sample represented by curve 22 was collected comparatively early in the run, that represented by curve 23 being collected at a later time. The small open circles 24 appearing on or near their respective curves indicate the boiling points and gravities of the 5% fractions, and since 95% of each of the two samples were distilled and collected, 19 of these 5% fractions are represented on each curve. Although curves 22 and 23 vary somewhat, due probably to changes in temperature conditions during the run or due to changes in the charge within the cracking still during its continued reduction, it is evident that the curves indicate compounds or fractions having similar properties as regards boiling

temperature and specific gravity. It will be noted with reference to Fig. 2 that substantially the greater portion of the 5% fractions included in the product boiling range have specific gravities ranging from around 0.75 up to 0.95, the high densities of the product constituents of the distillate, particularly among the higher boiling fractions, indicating the absence of substantial quantities of aliphatic and naphthenic compounds, which are characterized by comparatively lower specific gravity. Moreover, as previously mentioned, the cracked rosin distillates, like known aromatic compounds, are soluble in cold 96% sulphuric acid the aliphatic and naphthenic compounds being practically insoluble in this acid.

In order to indicate what compounds might be present in these cracked products, a number of known compounds having specific gravities and boiling point relationships near the points on these curves are also shown in Fig. 2 by the relatively large circles. Isoprene appears in the lower left hand corner and considerably out of proximity to the rosin curves, thus indicating that but little isoprene can be present in the distillate. It will also be noted that benzene (benzol) falls a considerable distance below the curves, benzene therefore not being present in the distillate in substantial amounts. Toluene, xylene and their substituted products such as ethyl benzene, normal and isopropyl benzene, santene, styrol, cymene, etc., fall on the curves. It thus appears that substantially the greater portion of the cracked products boiling below 450° F. is composed almost entirely of aromatic and aromatic substituted compounds, with the possible exception of a small amount of such substances as the heptenes, terpenes and possibly a few compounds boiling below 225° F.

The fraction of the total distillate comprising the product may be identified approximately as falling on the curves between the temperature limits of 100 to 450° F., although this temperature range is selected as the boiling point limits of the various grades of common motor fuels, it will be understood that under certain conditions it may be desirable to decrease the boiling range of the fuel within these temperature limits in accordance with given specifications. For instance, there is indicated in Fig. 2 the maximum boiling point of a particular grade of U. S. motor gasoline having an end point around 437° F.

In another run, the still 10 was charged with oil of turpentine and the latter distilled according to the preceding method described for the treatment of rosin. A representative sample of the cracked distillate was distilled in a Hempel fractionating column and the boiling point and specific gravities taken of 5% fractions as in the case of the

rosin distillate, the results of the tests on the turpentine fractions being indicated by curve 26 in Fig. 2. It will be noted that the turpentine distillate curve lies in the same region and is substantially coincidental with the lower portions of the rosin distillate curve 22, the lighter fractions of this particular sample of the turpentine distillate being somewhat more volatile than those of the 10 rosin products. The curve 26 indicates therefore that the cracked distillate derived from the oil of turpentine has properties characteristic of the aromatic and quite similar to the distillate obtained from rosin. Of the 15 sample tested, the lighter constituents of the turpentine product have the greater velocity, although it may be stated that the volatility of the rosin distillate may be increased as desired by causing more complete cracking 20 of the rosin vapors by regulating the temperature conditions in the superheater, the curves of course being merely typical of the product and not intended to define its boiling range. Due to the particular nature of the 25 samples and as represented by the curves in Fig. 2, the boiling temperatures of the lightest fractions are somewhat above the hereinabove specified initial boiling point which it may be desired that the product have, in 30 accordance with the initial points of certain commercial grades of gasoline. However, as stated, by varying the method of production, for instance the conditions of cracking, the volatility of the lighter fractions may be 35 regulated to give substantially any desired initial boiling temperature to the product. It may be preferred to carry out the method of production in a manner such that the volatility of the lightest fractions in the distillate 40 will correspond to the desired initial boiling points of the fuel product, and the distillate then fractionated in accordance with the end point of the product. Again, it may be desirable to carry out the cracking reaction to 45 such an extent that the heavier fractions of the distillate, that is those having boiling points above 450° F., may be broken down into fractions having boiling temperatures within the boiling range of the product.

50 **I claim:**

1. A non-detonating motor fuel composed of a mixture of gasoline and a liquid material comprising substantially a mixture of compounds of aromatic nature obtained by vaporizing rosin and cracking the vapors at a temperature between 600° F. and 1200° F., said liquid material having a boiling range within 100° F. to 450° F.
2. A non-detonating motor fuel composed of a mixture of gasoline and a liquid material comprising substantially a series of compounds of aromatic nature obtained by vaporizing rosin and cracking the vapors at a temperature between 600° F. and 1200° F., said liquid material having a boiling range

substantially within 100° to 450° F., and a specific gravity between 0.75 and 0.95.

3. As a product, a liquid material comprising a mixture of compounds of aromatic nature obtained by vaporizing rosin at substantially atmospheric pressure, and then in a subsequent operation cracking the vapors, the compounds of the mixture having specific gravities between 0.75 to 0.95, and a boiling range within 100° F. to 450° F.

70 75 80 85 90 95 100 105 110 115 120 125 130  
4. As a product, a motor fuel comprising substantially a mixture of compounds of aromatic nature obtained by vaporizing rosin at substantially atmospheric pressure, and then in a subsequent operation cracking the vapors, said mixture having a boiling range within 100° F. to 450° F., and a specific gravity between 0.75 and 0.95.

5. As a product, a motor fuel derived from rosin by heating and vaporizing said rosin and at substantially atmospheric pressure, subjecting the vapors to cracking at a temperature between 600° F. and 1200° F., and condensing the cracked vapors.

6. As a product, a motor fuel comprising a mixture of compounds of substantially aromatic nature obtained by vaporizing rosin at substantially atmospheric pressure, and then in a subsequent operation cracking the vapors, said mixture having a boiling range substantially within 100° F. to 450° F.

7. As a product, a motor fuel obtained by vaporizing rosin at substantially atmospheric pressure, and then in a subsequent operation cracking the vapors at a temperature between 600° F. and 1200° F., said fuel having a boiling range substantially within 100° F. to 450° F.

100 105 110 115 120 125 130  
In witness that I claim the foregoing I have hereunto subscribed my name this 11th day of July 1929.

DANIEL W. HOGE.